

[54] QUILTED FABRIC AND METHOD

[75] Inventors: **Bohumir Horeni, Hlavni; Vladimir Zid, Liberec; Bohuslav Neckar, Liberec; Jan Prochazka, Liberec**, all of Czechoslovakia

[73] Assignee: **Statni vyzkumny ustav textilni, Liberec, Czechoslovakia**

[22] Filed: **July 9, 1973**

[21] Appl. No.: **377,408**

**Related U.S. Application Data**

[63] Continuation-in-part of Ser. No. 847,194, Aug. 4, 1969, abandoned.

[30] **Foreign Application Priority Data**

Aug. 6, 1968 Czechoslovakia ..... 5696-72

[52] **U.S. Cl.** ..... 66/193; 112/412

[51] **Int. Cl.** ..... D04b 23/10

[58] **Field of Search** ..... 66/192, 193, 85 A; 112/412

| [56]                            | References Cited      |                      |          |
|---------------------------------|-----------------------|----------------------|----------|
|                                 | UNITED STATES PATENTS |                      |          |
| 2,158,006                       | 5/1939                | Ellis .....          | 66/193 X |
| 3,323,189                       | 6/1967                | Hayashi .....        | 66/193 X |
| FOREIGN PATENTS OR APPLICATIONS |                       |                      |          |
| 1,043,772                       | 11/1958               | Germany .....        | 112/412  |
| 512,488                         | 9/1939                | United Kingdom ..... | 66/192   |

Primary Examiner—Wm. Carter Reynolds

[57] **ABSTRACT**

A quilted fabric produced by increasing the number of courses per unit length so as to be at least eighty for each ten centimeters and based upon the tension of the reinforcing thread, the stitch formation, the filling coefficient and other factors so forming the shape of the loop so that it has a front loop portion which is substantially flat and a back loop portion which is substantially semi-circular.

10 Claims, 22 Drawing Figures



*Fig. 1**Fig. 2**Fig. 3**Fig. 4**Fig. 6**Fig. 5*



Fig. 10



Fig. 11



Fig. 12



SHEET 4 OF 7

Fig. 13



Fig. 14



Fig. 15



Fig. 16



Fig. 18



Fig. 17



PATENTED SEP 9 1975

3,903,714

SHEET 7 OF 7

Fig. 19



Fig. 20a



Fig. 20b



## QUILTED FABRIC AND METHOD

## RELATED CASE

This application is a continuation-in-part of our co-pending application Ser. No. 847,194, filed Aug. 4, 1969, now abandoned, to which reference is made for any disclosure, amplifying, extending or supplementing the contents hereof and such disclosure is incorporated herein as if more fully set forth here.

## BACKGROUND OF THE INVENTION

The present invention relates to the quilting of a fleece, batt or fibrous webbing and more particularly to the production of improved quilted fabrics.

Stitch-bonded or knitted quilt fabrics of natural or synthetic fibers are well known and extensively used. In such fabrics, a web of fibrous material, either as fleece, sandwich batt, or monofilament yarn is reinforced by one or more binding networks of warp stitching to produce a fabric having a plurality of symmetrical or uniform tufts filled with fibrous material. The most common networks used are single warp or chain stitch, tricot stitch or combinations thereof in a network, not exceeding 60 wales per 10 cm and 80 courses per 10 cm.

It has been found that conventionally stitched quilted fabrics have poor structural properties exhibiting a severe lack of tensile strength and slippage of the fiber at the binding points. As a result, the slightest tension causes a permanent deformation of the tuft, which during wear allows bulging of the fabric at stress and flex points, such as knees and elbows, low resistance to abrasion; tendency to pill and, in pile or raised fabric, to shed. Conventionally stitched quilted fabrics also exhibit poor ability to anchor or clamp the fiber bundles, within the loop, resulting in extremely low resistance to transverse tension and actual loss of fibers from the fill. These situations appear to arise or be caused either by an insufficient number of courses, the improper shaping of the tuft loop, or by the application of insufficient tension on the thread, producing as a consequence a low co-efficient of tuft filling which may be defined as the ratio between the sum of fiber cross section areas in a stitch loop and the total area confined by the stitch loop. Consequently, the fabric produced by conventional methods is limited to such uses as insulating material, textile laminate backings and decorative fabrics, all of which are subject to little, if any, exposed wear.

It is the object of the present invention to provide quilted fabrics in which the disadvantages enumerated above are non-existent.

It is another object of this invention to provide quilted fabrics having such degree of quality as to be readily usable as outwear clothing and in other applications where strength, form and shape are required.

It is a specific object of the invention to provide a quilted fabric wherein the co-efficient of tuft filling is increased, the loop shape stabilized and the stitch bonding point strengthened.

According to the present invention a quilted fabric is produced by increasing the number of courses, the thread tension, and the shape of the loop in a predetermined and defined manner dependent upon its weight, specific gravity and the thickness of the fibrous web fill.

It has been found that quilted fabric made according to the present invention will have a considerably higher strength, a greatly suppressed tendency to bulge as well as a higher fiber anchoring than conventional fabrics.

Spontaneous fiber shedding or pilling during wear will also be markedly reduced even if the fabric is raised or pilled. The fabric produced by the present invention rivals more common fabrics, such as sateens, regular knits, etc. and may be used in such new applications as in outerwear, underwear, furnishings and beddings as well as in a variety of industrial uses. Above all, the fabric is simple to produce, having a low production cost and high production rate on readily available conventional machines.

## BRIEF DESCRIPTION OF THE DRAWINGS

The above objects and advantages, as well as others, together with a detailed description of the invention, will be seen from the following description taken with regard to the annexed drawings in which:

FIG. 1 is a schematic representation along a longitudinal section showing the loop formation and tuft structure of successive courses in a single wale of conventionally stitched fabrics, while the same remain on the knitting machine;

FIG. 2 is a view similar to FIG. 1 showing the fabric of FIG. 1 in relaxed condition and removed from the knitting machine;

FIG. 3 is a view similar to that of FIG. 1 wherein a stable loop is formed in accordance with the present invention;

FIG. 4 is a view similar to that of FIG. 3 showing a modified fabric according to the present invention;

FIG. 5 is a perspective view of a portion of a fabric of the type shown in FIGS. 1 and 2;

FIG. 6 is a perspective view similar to FIG. 5 showing a portion of a fabric of the type shown in FIG. 4;

FIG. 7 is a perspective view of fabric made with a battening interior in accordance with the present invention;

FIG. 8 is a view similar to that in FIG. 7 showing the application of a combined chain stitch and tricot stitch network;

FIGS. 9a-9c show schematic views of a needle stitch mechanism employed to provide the present invention;

FIG. 10 is a schematic view of a needle stitch mechanism and quilting machine elements employed to provide the fabric of this invention;

FIG. 11 is a graph of the course of the coefficient of stitch loop filling;

FIG. 12 is a graph of the course of the coefficient of stitch loop filling when transverse deformation of fiber profiles arises, curve a and the corrected curve b;

FIG. 13 is an illustration of the loop stitch of the invention showing that the upper side of the loop is constituted by two yarn ends with the force 2F acting on the upper part of the loop and the lower side of the loop constituted by one yarn end with the force F acting thereon;

FIG. 14 is an illustration of the stitch loop shape below the stability limit;

FIG. 15 is a diagrammatic illustration of the formula  $G_r = G/N$  for determining the fiber weight in a single course;

FIG. 16 is a diagrammatic illustration of the stitch loop shape at the stability limit when the lower loop stitch arch is semi-circular;

FIG. 17 is a diagrammatic illustration of the stitch loop shape above the stability limit;

FIG. 18 is a diagrammatic illustration of the formula,  $D = (1/N) - (D_s / \cos \psi)$  where the loop stitch is below the stability limit;

FIG. 19 is a diagrammatic illustration of the formula,  $D = (1/N) - D_r$ , for determining the knit course number for stitch loops at and above the stability limit; and

FIGS. 20 (a) - (b) are diagrammatic illustrations for determining the length of the chain stitch yarn. 5

#### DESCRIPTION OF PREFERRED EMBODIMENTS

Turning to FIGS. 1, 2 and 5, which, it will be recalled, show a conventionally formed fabric, there is seen a plurality of coursewise tufts T formed of fibrous web W, reinforced by a plurality of simple chain stitch thread 1 bound respectively at points A, all lying along a common axis. Each of the tufts T, of this fabric, are of an elongated elliptical cross section; that is, the upper thread portion L<sub>1</sub>, is substantially equal to the lower thread portion L<sub>2</sub> and the cross sectional surface P of the ellipse has substantially equal upper and lower portions 2 and 3 respectively. The fabric even in its relaxed state, as seen in FIG. 2, is not significantly altered, in its shape, although each tuft T does become somewhat more round having a total surface P<sub>1</sub> somewhat larger than its original surface P as seen in FIG. 1. The loop portion L<sub>1</sub> and L<sub>2</sub>, as well as the surface portions 2 and 3, nevertheless remain substantially equal to each other. Such an elliptical body is highly elastic since any pull on its fabric will cause it to elongate and the loops L<sub>1</sub> and L<sub>2</sub> to straighten along the axis a. Thus, as tension is applied to the fabric the loops readily change shape causing the binding points A to loosen, shift position and permit the web filling to be dislodged. It will also be observed that the filling coefficient m of the conventionally formed fabric (FIG. 5) is extremely poor since the ratio between the sum of fiber cross-section areas in a stitch loop and the total area confined by the stitch loop is small, consequently the force F, necessary to pull a fiber from the tuft is minimal and that transverse deformation is quite high. The end result of course is a fabric which has the disadvantages enumerated in the introduction hereto. 15

We have found that a stable quilted fabric is formed by establishing the number of courses based upon certain of the processing parameters, as for example, those relating to the stitch formation, number of wales and thread tension. As will be described in greater detail hereinafter, changes or modifications can be made so that the process may be adapted to any conventional warp quilting machine, as for example, that shown in U.S. Pat. No. 3,310,964 issued Mar. 28, 1967 to E. Peschl et al.

These parameters have been embodied in a formula wherein any fibrous web having a weight of up to 600 grams/square meter can be reinforced with a network of threads in any warp stitch construction wherein the network comprised a number of courses per each 10 cm at least equal to N, N being determined by the equation 10

$$N = \frac{7589.46}{\sqrt{T}} + 100 B \quad \left( 1 - \sqrt{1 + \frac{51.79}{B \cdot \sqrt{T}}} \right)$$

where B is determined by the equation

$$B = \frac{2.88 \cdot G}{T \cdot m \cdot \gamma \cdot (0.483 + \alpha)}$$

wherein

G = weight in g/sq.m of the fibrous web to be processed

T = binding thread titre in denier

$\gamma$  = specific gravity in g/cu. cm of the fibers in the web

m = the constant equalling 0.40 representing the filling coefficient of the material

$\alpha$  = the constant which with the fibrous web weight up to 200 g/sq.m equals zero while with the fibrous webs of weight range of from 200 to 600 g/sq.m. is determined by the equation

$$\alpha = 0.002 \cdot G - 0.400$$

and represents machine operating factors such as thread tension, winding tension etc.

In order to appreciate the significance and the derivation of the above formula the following basic principles of binding yarn feeding and tension are set forth and the derivation of the formula per se is set out.

Within each operating cycle of the stitch-bonding process as shown in schematic FIGS. 9a, 9b and 9c, a certain predetermined binding yarn length is supplied to the stitch forming organs, or in other words, the supplied yarn length in any given case is the same or constant within each operating cycle. This is achieved by the fact that within each operating cycle the yarn package from which the binding yarn is wound off turns by a predetermined angle, thus dispensing the aforesaid constant binding yarn length. 20

Referring now more particularly to FIG. 10, the constant binding yarn supply proceeds as follows:

The rotation of the warp beam 31, that is, the binding yarn package, is controlled by a let-off motion 32 comprising a plurality of gears designed to transmit the movement from the main machine shaft up to the warp beam. The rotational movement is divided in the let-off motion into two components which, if added or subtracted in a differential, will give the resulting continuously controllable warp beam rotation rate. 25

The control of the differential gear performance is based upon the position of a tension controlling rod 33 and transmitted via a crank lever 34 and a connecting rod 35 to the let-off motion 32.

Thus, the position of the tension controlling rod 33 affects the yarn feeding rate.

For example, with a fully wound warp beam, the tension controlling rod is in the position 33' so that the beam rotation will be slower than in position 33'' wherein the warp beam is almost empty and will rotate at higher speed. Consequently, in this manner in the two cases mentioned the respective lengths of let-off warp or binding yarns remain the same. 30

Apart from the aforementioned constant yarn length, the tension controlling rod makes it possible to take off, within each operating cycle, a necessary surplus length of binding yarn, which length, after the cycle has been closed, is retracted or taken up again by the action of the tension controlling rod. 35

Such a pulsating or oscillating yarn feeding system operates as follows:

In the yarn tension controlling mechanism described above which comprises the tension controlling rod 33, crank lever 34 and connecting rod 35, a certain play is provided, enabling the tension controlling rod 33 to oscillate within limits during the stitch loop formation and to act at the same time as a consumed yarn length compensator. The play is denoted in FIG. 10 by refer-

ence symbol  $a$  is relatively small and cannot influence the position of the differential of the yarn feeding rate.

The entire aforementioned process of both constant and oscillating feeding within the stitch-bonding cycle takes place under a preadjusted binding yarn tension.

This tension is adjusted as follows:

On a shaft 36 carrying the tension controlling rod 33 and the crank lever 34 there is provided a helically wound flat spring (not shown) of which one end is attached to the shaft 36 while the other bears upon a stationary abutment arranged on the machine sidewall.

The spring end portion is not fixedly attached to the shaft 36 but rather adjustably by means of an adjusting ring (not shown) so that the torsion of the spring can be reduced or, on the contrary, increased, thereby making it possible to control the entire warp yarn tension.

#### Coefficient of Stitch Loop Filling

From a purely theoretical standpoint the dependency of the stitch loop filling coefficient  $m$  upon the yarn tension  $F$  cannot be justified since

$$m = m(F)$$

where the function  $m(F)$  increases together with increasing quantity  $F$ . Since the filling coefficient  $m$ , for principally physical reasons, has to vary within interval  $0 \rightarrow 1$ ,  $m \rightarrow 0$  corresponds to  $F \rightarrow 0$  and  $m \rightarrow 1$  theoretically corresponding to the theoretical quantity  $F \rightarrow \alpha$ . Moreover, since the function  $m(F)$  has, for principally physical reasons, within the entire interval  $P \leftarrow (0, \rightarrow \alpha)$  a positive derivative, the function  $m(F)$  can be schematically plotted as in FIG. 11.

No substantial physical reasons can be found for the above relation being discontinuous in the first derivative, or for the understanding of inflection points therein.

The relation  $m(F)$  shown in FIG. 11 holds until a transverse deformation of fiber profiles occurs.

The curve  $m(F)$  involving this deformation factor has a different course, particularly for higher  $F$  quantities, as shown in FIG. 12 by  $a$  and where the corrected curve is indicated by  $b$ .

No substantial physical reasons exist for which the relation might be considered as discontinuous in the first derivative, and for which it might involve an inflection point.

It is to be noted that the two curves have a converging limit for  $F \rightarrow \omega$  towards  $m \rightarrow 1$  but that the corrected curve  $b$  will acquire linear course much sooner, since except for the lowest values  $F$ , the second derivative is lower.

From the viewpoint of practical determination of the function  $m(F)$ , this fact means that a relatively broad interval  $(X, Y)$  of the force  $F$  the relation can be expressed with sufficient technical preciseness as

$$m(F) \triangleq m = \text{const.}$$

The aforementioned expected facts have been fully proven by experimental research work.

In this experimental work, a plurality of webs of various orientation and specific weight were stitchbonded in varying knit-course densities and under varying warp yarn tensions under strict laboratory conditions. The filling coefficient was evaluated by conversion from experimentally found quantities, such as, besides others, the number of knit-courses in the taut fabric immedi-

ately behind the needles, and in appropriately treated released fabric.

It has been found that within the examined warp yarn tension interval which was kept during the experiment at many times higher and lower than that allowed by practical technological conditions, the filling coefficient of the fabric behind the needles is practically independent of the yarn tension, and web orientation.

Likewise, no influence of web weight on the quantity  $m$  was observed.

On the other hand, the filling coefficient  $m$  in released and treated fabrics is markedly dependent on the selected knit-course number, it being, in the case of a lower course number than disclosed in the above formula, always lower than the substantially constant coefficient in the taut fabric just behind the needles.

In case of the disclosed course number and higher course numbers, no difference between the coefficients was found in practice.

In summary, it can be stated that:

a. the relation  $m = m(F)$  is not pertinent from a purely theoretical viewpoint;

b. the course of the function  $m = m(F)$ , however, is within a practically used yarn tension interval, "flat" and practically indistinguishable from the formula  $m = m(F)$  where  $m$  equals a constant, it being understood that the experimentally examined yarn tension interval was both above and below the yarn tension interval employed;

c. the statement in paragraph (b) holds also for webs of various specific weights and orientations;

d. the filling coefficient found with all types of fabric behind the needles and with released and treated fabrics having the same and higher knit-course numbers than that disclosed in the above formula has varied within a narrow interval of about  $m = 0.4$ .

#### Stitch Loop Geometry of Chain Stitch Structures

Practical examination of stitch cross-section has proved that the stitch loop has not a circular but rather a substantially unsymmetrical elliptical configuration.

The stitch loop is constituted on the upside by two yarn ends and on the underside by one yarn end as shown in FIG. 13.

Assuming that the interval tension of the binding threads is the same in all regions, then the force  $2F$  acts in the upper part of the stitch loop, whereas in the lower part thereof only the force  $F$  acts.

The stitch loop shape below the stability limit is shown in FIG. 14.

There results from the mathematical calculation of the relations involved in FIG. 14 the following:

$$\cos \Phi = \frac{\frac{D}{2}}{R}, \quad R = \frac{D}{2\cos \Phi}$$

$$\cos \Phi = \frac{\frac{D}{2}}{r}, \quad r = \frac{D}{2\cos \Phi}$$

From the equilibrium of vertical components of forces acting at the point B, it may be deduced that

$$2F \cos \Phi = F \cos \psi$$

If inserting the preceding relations into the last mentioned equation, the result is that

$$2 \frac{D}{2R} = \frac{D}{2r}$$

where from

$$R = 2r$$

Thus, the radius of curvature of the upper branch of the stitch loop (1) is double the radius of the lower stitch loop branch (2).

The filling coefficient  $m$  may be defined as a relation between the sum of fiber cross-section areas in a stitch loop ( $P_r$ ) and the total area confined by the stitch loop ( $P_c$ ) so that

10

or

15

$$m = \frac{P_r}{P_c}$$

It is to be understood that in order to find the filling coefficient  $m$  the aforementioned quantities have to be known.

If we insert for the weight of a unit web element ( $g/sq.cm$ ) the symbol  $G$  and for the density of courses per unit length (1 cm) the symbol  $N$ , the fiber weight in a single course ( $G_r$ ) will result from the following relation (see FIG. 15):

$$G_r = \frac{G}{N}$$

If  $P_c$  (sq.cm) is the total area confined by the stitch loop in a single course (FIG. 15) the specific weight of compressed web element in the loop can be calculated from the following formula

30

$$P_r = R^2 \left( \frac{\pi}{2} - \Phi \right) - \frac{1}{2} DR \sin \Phi +$$

$$r^2 \left( \frac{\pi}{2} - \psi \right) - \frac{1}{2} Dr \sin \psi$$

35

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

The loop stitch cross-section area  $P_c$  is derived as follows:

The segment area  $P_R$  bounded by the arch of radius  $R$  and by the line segment  $AB$  (i.e. the upper segment of the circle) is given by the following mathematical relation:

$$P_R = \frac{\pi R^2}{2\pi} \cdot 2 \left( \frac{\pi}{2} - \Phi \right) = \frac{D}{2} R \sin \Phi$$

or

From the foregoing equations for  $P_R$  and  $P_r$ , the total area  $P_c$  of stitch loop is found to be the sum  $P_R + P_r$  or

$$P_r = R^2 \left( \frac{\pi}{2} - \psi \right) - \frac{1}{2} DR \sin \psi$$

The stitch loop shape at the stability limit is a particular case of the general stitch loop shape wherein the center of a circle of radius  $r$ , i.e. the point  $S_2$ , has descended into the point  $O$  and become identical therewith. In this case the lower stitch loop arch becomes a semicircle as shown FIG. 16.

For this particular case the following relation holds:

$$r = \frac{D}{2}; \quad R = D$$

and it further holds:

$$\cos \Phi = \frac{2}{D} = \frac{1}{2}; \quad \Phi = \frac{\pi}{3}; \quad \sin \Phi = \frac{\sqrt{3}}{2}$$

$$\cos \psi = \frac{2}{D} = 1; \quad \psi = 0; \quad \sin \psi = 0$$

After substitution of the foregoing relations into the formula for the calculation of  $P_c$ , it is seen that

$$P_c = D^2 \cdot 0.483$$

In regard to the stitch loop shape under the stability limit the following relations hold:

$$N = \frac{G}{m\gamma P_c}$$

or eventually

$$\psi < 0 ; \cos \psi \cos \psi 1$$

Thus, for instance, for  $\psi = 20^\circ$ ;  $\cos \psi = 0.93969$ ;  $\sin \psi = 0.34907$   
and further

$$\sin \psi = 0.34202$$

or

$$r = \frac{D}{2 \cdot 0.93969} = \frac{D}{1.88}$$

or, assuming that it holds that

$$R = 2r = 2 \cdot \frac{D}{1.88} = 1.063D$$

wherefrom

$$\cos \phi = \frac{D}{2 \cdot 1.063D} = 0.471; \phi = 62^\circ$$

or

$$\sin \phi = 1.0821; \sin \phi = 0.88295$$

After insertion of the aforesaid quantities into the equation for the determination of  $P_r$  the following formula is obtained

$$P_r = D^2 \cdot 2 \cdot 0.340$$

The stitch loop shape above the stability limit (i.e. also a stable shape) is shown in FIG. 17.

The total stitch loop area  $P_r$  is given in this case by the relation:

$$P_r = D^2 \cdot 0.483 + Da$$

if putting  $a = \alpha D$ .

the following formula will be obtained:

$$P_r = D^2 (0.483 + \alpha)$$

After substitution of the last mentioned formula into the equation for the calculation of knit-course number  $N$ , that is

$$N = \frac{G}{m P_r \gamma}$$

the following formula is obtained:

$$N = \frac{G}{m D^2 (0.483 + \alpha) \gamma}$$

Further for  $D$  below the stability limit the following relation shown in FIG. 18 holds:

$$D = \frac{1}{N} - \frac{D_r}{\cos \psi}$$

Since, however, it is necessary to determine the knit-course number  $N$  for the stitch loops at the stability limit,  $D$  can be calculated from the relation:

$$D = \frac{1}{N} - D_r$$

as shown in FIG. 19 and wherein  $D_r$  = binding yarn diameter. The foregoing formula is to be substituted into the equation for determining the quantity  $N$ .

5 After substitution and simplification the following formula results:

$$10 \quad N^2 D_r^2 - N \left( 2D_r + \frac{G}{(0.483 + \alpha) m \cdot \gamma} \right) + 1 = 0$$

After inserting an auxiliary quantity  $A = (0.483 + \alpha) m \cdot \gamma$  there is obtained for the solution of the foregoing quadratic equation the following relation:

$$15 \quad N = \frac{1}{D_r} + \frac{G}{2AD_r^2} \pm \sqrt{\frac{G^2}{4A^2D_r^4} + \frac{G}{AD_r^3}}$$

20

After inserting another auxiliary quantity  $B = G/2A \cdot D_r^2$  the following formula is obtained:

$$25 \quad N = \frac{1}{D_r} + B \pm \sqrt{B^2 + B \frac{2}{D_r}}$$

Since the negative sign only has the physical sense it holds further that

$$30 \quad N = \frac{1}{D_r} + B \left( 1 - \sqrt{1 + \frac{2}{BD_r}} \right)$$

35 wherein  $B = G/2AD_r^2$  and as  $A = (0.483 + \alpha) m \cdot \gamma$  so that

$$40 \quad B = \frac{G}{2D_r^2} \cdot \frac{1}{(0.483 + \alpha) m \cdot \gamma}$$

Further for the calculation of the binding yarn diameter the following relations hold:

$$45 \quad D_r = \frac{1.25}{\sqrt{cm}} = \frac{1.25}{\sqrt{9000}} \sqrt{T} = 0.013176 \sqrt{T}$$

$$\frac{D_r^2}{1} = \frac{0.0001736 \cdot T}{75 \cdot 8946}$$

$$50 \quad D_r = \sqrt{T}$$

After inserting the above quantities  $D_r$  into the foregoing equations for  $N$  and  $B$ , respectively, the following formula is obtained:

$$55 \quad N = \frac{75 \cdot 8946}{\sqrt{T}} + B \left( 1 - \sqrt{1 + \frac{151.79}{B \sqrt{T}}} \right)$$

in which

$$60 \quad B = \frac{2880.02G}{T} \cdot \frac{1}{(0.483 + \alpha) m \cdot \gamma}$$

65 Since in practice the weight of the stitch-bonded web is expressed mostly as weight of 1 sq.meter in grams ( $G$  [ $g \cdot m^{-2}$ ]) and the knit-course number  $N$  per 10 cm (1 dm), the following final formula is obtained

$$N \left[ \text{dm}^{-1} \right] = \frac{7589.46}{\sqrt{T}} + 1000B \left( 1 - \sqrt{1 + \frac{151.79}{B \sqrt{T}}} \right) \quad \text{or}$$

in which

$$B = \frac{2.88G \left[ \text{g.m}^{-2} \right]}{Tm\gamma(0.483 + \alpha)} \quad 10$$

which formula is the same as set forth above and wherein

$G$  = weight of 1 sq.meter of the stitch-bonded web in grams

$T$  = titer of the binding yarn in denier

$\gamma$  = specific gravity of the fibrous layer in g/cu.cm.

$m$  = filling coefficient which equals 0.4

$\alpha$  = stability coefficient which the fibrous layer weight up to 200 g/m<sup>2</sup> is zero so that it is fully sufficient to make stable fabrics up to aforementioned

fibrous layer weight on the stability limit, and which for fibrous layers within the weight range of from 200 to 600 g/sq.m is given by the formula

$$\alpha = 0.002G - 0.400 \quad 25$$

which means that within said weight range the stable fabrics are manufactured above the stability limit.

The foregoing conclusions are complemented with the following statements:

If it is indicated that:

the  $P_c$  of fabrics under the stability limit is  $P_{c_{ps}}$ ;

the  $P_c$  of fabrics at stability limit is  $P_{c_{ms}}$  and

the  $P_c$  of fabrics above the stability limit is  $P_{c_{ns}}$ ,

we will find that in the stitch-bonding process for the same course density  $N$ , the following relation holds:

$$P_{c_{ps}} < P_{c_{ms}} < P_{c_{ns}} \quad 40$$

Thus in the stitch-bonded fabric below or under the stability limit, when removed from the machine and appropriately treated, is then allowed to relax,  $m$  is rendered lower than 0.4 and consequently the use value of the respective fabric is unfavorably affected.

This release is enabled by the length of the chain stitch yarn, as hereinafter explained.

The length of the chain stitch yarn can be derived from FIGS. 14 to 20, and particularly from FIGS. 19 to 20. For this length the relationship is

$$l_c = 4 \left( R + \frac{D_r}{2} \right) \left( \frac{\pi}{2} - \Phi \right) + 2 \left( r + \frac{D_r}{2} \right) \left( \frac{\pi}{2} - \psi \right) \quad 45$$

This length, however, should be slightly increased, since the binding yarn surrounds in the point B (see FIGS. 13 and 14) two binding yarns, as can be seen in FIG. 20.

In practice, two modes of encircling are possible, i.e. 20a or 20b. Thus, it is necessary to add to the length  $l_c$  either  $\pi D_r$  or  $(\pi D_r + D_r)$ . Since the respective encircling mode cannot be predetermined, an average quantity for  $l_c$  has to be introduced into the formula, such quantity equalling

$$(\pi + \frac{1}{2}) D_r = 3.64 D_r \quad 65$$

Thus, the total binding yarn length necessary for the chain stitch loop results from the following relation

$$l = l_c + 3.64 D_r$$

$$l = 4 \left( R + \frac{D_r}{2} \right) \left( \frac{\pi}{2} - \Phi \right) +$$

$$2 \left( r + \frac{D_r}{2} \right) \left( \frac{\pi}{2} - \psi \right) + 3.64 D_r$$

10

To determine the stitch loop length for the stitch at the stability limit there is obtained for 1 the following relation:

$$l = 3.67 D + 6.26 D_r$$

To determine the stitch loop length for the stitch below the stability limit, as by using the aforesaid example where

$$\phi = 62^\circ \text{ and thus } \text{arc } \phi \doteq 1.082; R = 1.063 D \text{ and } \phi = 20^\circ \text{ and thus } \text{arc } \psi \doteq 0.349; r = D/1.88$$

there is obtained for 1 the following formula:

$$l = 3.38 D + 5.84 D_r$$

Finally, to determine the stitch loop length for the stitch above the stability limit there is obtained for 1 the following formula:

$$l = (3.67 + 2X) D + 6.26 D_r$$

The fabric release, however, cannot occur with fabric on stability limit and with fabrics above stability limit either. Nevertheless the manufacture of fabrics above stability limit is not recommended, since the increased knit-course number unfavorably influences the machine productivity.

When multi-warp stitch constructions are used, e.g., with  $n$  (being more than one) warps containing different denier yarns, the total denier will be calculated from the equation

$$T = \frac{(\sqrt{T_1} + \sqrt{T_2} + \dots + \sqrt{T_n})^2}{n}$$

While the lowest course density obtaining the required wear properties, as discussed above, will, of course, result from the maximized combination of the materials used and from their determining properties, it is believed that the greatest number of courses  $N$  should not, in practice, exceed 300 per 10 cm.

Employing the above formulation, novel quilted fabrics exhibiting enhanced wear qualities are obtained. Two such fabrics, similar to each other, are shown in FIGS. 3, 4 and 6 wherein the fabric is reinforced with a thread 1 bound at points A lying along the common axis  $a$  in which the upper loop portion  $L_3$  is considerably shorter than the lower loop portion  $L_4$ . The fabric shown in FIGS. 4 and 6 differ from that shown in FIG. 3 in that the loop binding points A are vertically elongated, giving it a somewhat longer inner loop.

The fabric thus produced provides a lower loop portion  $L_4$  substantially semi-circular in cross section and an upper loop portion  $L_3$  having a more or less substantially flat contour. The cross-sectional surface or area  $P_2$  is also considerably larger than the cross-sectional surface or area  $P_3$ . As will be obvious, a by any pull

along axis *a* will cause only limited movement of the loops because the upper loop portion *L<sub>3</sub>* defines the extent of such movement. The tuft loop can only be elongated so far as the upper loop portion *L<sub>3</sub>* can be made to coincide with the axis *a* and since it is already substantially flat, movement is very small. Consequently, virtually no significant loosening of the loops at the binding points *A*, shifting of the threads or dislodging of web filling occurs.

Diagrammatic comparison of the improvement in the filling coefficient will be seen from FIG. 6 where it is obvious that the filling coefficient is greater than that shown in the conventional fabric of FIG. 5. Consequently, the *F<sub>2</sub>*, necessary to pull out a fiber from its bundle (FIG. 6), is considerably higher than the force *F<sub>1</sub>* (FIG. 5). In the fabric of the present invention, the coefficient *m* is at least 0.4 and often *F<sub>2</sub>* is so high as to approach or exceed its strength of the fiber itself. This results in considerable lowering of deformation due to the crosswise stressing of the fabric and in an important increase of fabric strength in its transverse direction.

As an example of the versatility of the present invention, reference is made to FIG. 7 showing a quilted fabric of layered material reinforced by one warp end system in chain stitch construction. The fabric has a fibrous web 4 comprising a plurality of layers 5 all having fibers transversely arranged relative to the axis of the fabric. The web 4 is reinforced by parallel rows of interconnected face loops 6 and back loops 7 arranged in chain stitched wales 8. For the purpose of example, a setting of 40 wales for each 10 cm with 100 courses per 10 cm length was employed. The back loop 7 penetrates through the web 4 from the binding point *A* which, as will be seen, lies substantially at the front face of the fabric. Because of the tension placed on the reinforcing thread, its front loop 6 tends to indent the fabric creating something of a valley between two adjacent hills or mounds 9 centrally between the adjacent wales 8. As a result a quilted fabric having a ribbed or corduroy appearing surface along the successive mounds 9 is formed. The back or reverse face is similarly formed. It will be appreciated that when a greater number of courses are employed the shape of the faces will be closer to those shown in FIGS. 3, 4 and 6.

Another variation is shown in FIG. 8. This fabric is similar to that shown in FIG. 7, except that the reinforcing thread is made into a network of combined chain stitches and tricot stitches. In FIG. 8, the tricot stitch is indicated by dot and dash line 10 which forms a portion of the stitch structure on its back face. Thus, the tricot thread leaves back loop of wale 8 after it penetrates the web 4 and passes over to the adjacent wale 8' where it interlaces with the thread of that wale to form the loop 6' of the next course. In the next stitch, the tricot thread forms the back loop 10' and returns to its initial wale 8 where it subsequently forms the loop 6'' of the third or next succeeding course. The back loops 7 of the simple chain stitch interlace as they did in the construction of FIG. 7.

The combined chain and tricot stitch construction of FIG. 8 changes the fabric in that the corduroy or ribbed effect on its reverse face is suppressed, while the front face remains the same. The fabric thus produced has a corduroy effect on one side and a smooth effect on the reverse side. Since two warp systems are used to form the network, this reinforced thread is stronger and the tendency for the fabric to unravel is reduced. The fab-

ric also has a stronger tensile strength since the tricot thread passes to and fro between adjacent wales.

The quilted fabrics, according to this invention, may be produced on any conventional quilting machines. 5 One such machine being described in full in the aforementioned patent — U.S. Pat. No. 3,310,964. These machines may be one or multibar flat warp knitting machines equipped with compound or two-part needles provided with piercing points and the hooks of which 10 are provided with latches slidably mounted within the needle stems. The needles and the latches are mounted in needle and latch bars, respectively, which are driven in usual manner from a common drive shaft. The needles cooperate with lapping guide units which are fitted 15 with lapping guides mounted on guide bars moving transversely in holders which, similarly as the needles and latches, are driven from the main drive shaft. Operation of this machine proceeds in the conventional manner. A quilting machine, however, unlike the conventional warp knitting machine, guides the fibrous web on a stationary knockover table and amovable web holder table, which motion carries the web. The web holder table is movable from the main shaft.

20 The quilting machine is further equipped with a conveyor means for supplying the fibrous web to the knitting mechanism between the knock-over and web holder tables. Warp beams are arranged on the machine in a known manner for feeding and unwinding the binding thread. The take-up means selvedge trimmers, etc. are also supplied. The fibrous web may be prepared on a web forming machine of the cotton, wool or flax types, and it is superimposed in layers on any known web-laying equipment, such as the Blamier's lap forming apparatus, to obtain the required thickness or 25 weight.

In the production of a quilted fabric according to the invention (FIGS. 9a - 9c) the conveyor system 13 carries the fibrous web 4 between the stationary knock-over table 11 and the web holder table 12 to cross the path of the needles 14. The needles 14 reciprocate from their rear position forward, they pass between the two tables 11, 12, penetrating at the same time the fibrous web 4 which is held by the web holder table 12. 30 The needles 14 complete their movement to their rear-most position where the binding threads 15, 15' are lapped on their hooks by the lapping guides 16, 16' (FIG. 9b). The needles 14 then return, their hooks being colsed by the sliding latches 17, and pull the 35 loops formed of the binding warp ends 15, 15' through the fibrous web 4 and the previously formed loops (FIG. 9c). Thus, new loops are formed and the old loops are knocked over the heads of the needles 14 as they return to their rear position. As soon as the needles 14 have returned, the produced fabric length is 40 drawn off. The fabric length to be drawn off depends on the given number of courses in the fabric.

45 The stitch construction - in our case a two-bar construction - is preset by adjusting the movement of the lapping guides 16, 16' in the manner known with conventional warp knitting machines, and by threading these lapping guides.

50 It will be obvious from the foregoing that among the novel features of the present invention is the use of a substantially increased number of courses per unit length, increased tension of the thread itself, a new shape to the loop structure and the maintenance of the binding point, or knock-over point at or substantially 55

near one of the faces of the fabric. It is these factors which individually and jointly provide one or more of the advantages enumerated above and provide fabrics which are stronger, more durable, more attractive and of wider use than heretofore. With this in mind, it will be appreciated that the invention may be employed to provide a variety of differently appearing quilted fabrics and with a variety of different materials.

Any stitch structure or network may be employed in addition to the simple chain and tricot stitches shown, 10 as for example double tricot, double sateen. In the simplest quilted fabrics, a single warp, simple chain stitch construction may be used to reinforce the fibrous web lengthwise while the laying of the fibers crosswise in the web may be relied upon for transverse stability. This 15 type of quilted fabric can be used mainly for insulation purposes where the strain may be exposed to is not considerable. If some additional transverse strength is required, the web may be reinforced in either tricot or sateen stitch constructions or double warp stitch construction. With a double warp stitch construction, neither unravelling nor loosening of the fibrous web can occur.

The fibrous web may be made of monofilament, fibrillated or other forms of natural, man-made, or inorganic fibers, or blends thereof. It is also possible to use a sandwich web comprising different materials and the web may be of isotropic anisotropic character. The fibers should as a rule, however, be arranged crosswise in the fabric as noted above. The weight of the fibrous web may be less than 50 g/sq.m although it may be four to twelve times higher if desired. The type of fibers or their blends or the sandwich combinations may be chosen to suit the required wear properties or end uses of the finished product. The binding thread may be either a spun yarn, single or plied, a monofilamentary or plied filament yarn, both natural or man-made. For the most part, cotton, viscose, wool or blended fibrous webs should reinforce or stitch-bond with polyamide, 20 polyester or viscose filament yarn warps.

As examples of the versatility of the present invention, there follows a number of examples (for illustration only) wherein the present invention is employed to provide improved fabrics. The execution of each example was performed on conventional equipment and in accordance with the concepts taught herein and the resultant fabric was tested for each of the suggested end uses.

#### EXAMPLE 1

50

Fibrous web of 2.5 den., 60 mm viscose staple  
Specific weight  $\gamma = 1.52$ , weight  $G = 70$  g/sq.m  
Two-bar stitch construction tricot + tricot, opposite  
lapping  
Binding thread: Viscose filament yarn  $T = 60$  den., on  
both bars  
Wale set: 80 per 10 cm  
Course set:  $N \geq 239.5$  per 10 cm  
(filling coefficient  $m = 0.4$ ,  $\alpha = \phi$ ,  $B = 11.44$ )  
Suitable end uses: print backings, shirtings

#### EXAMPLE 2

Fibrous web of cotton fibers  
Specific weight  $\gamma = 1.55$ , weight  $G = 150$  g/sq.m  
Two-bar stitch construction chain stitch + tricot  
Binding thread: polyamide filament yarn  $T = 90$  den.  
on both bars

Wale set: 60 per 10 cm  
Course set:  $N \geq 137.1$  per 10 cm  
( $m = 0.4$ ,  $\alpha = \phi$ ,  $B = 16.03$ )

5 Suitable end uses: children's wear, coats and over-coats, industrial fabrics

#### EXAMPLE 3

Fibrous web of wool fibers  
Specific weight  $\gamma = 1.36$ , weight  $G = 300$  g/sq.m  
Two-bar stitch construction chain stitch + tricot  
Binding thread: texturized polyester filament yarn  $T = 120$  den. on both bars  
Wale set: 50 per 10 cm  
Course set:  $N \geq 92.9$  per 10 cm  
( $m = 0.4$ ,  $\alpha = 0.2$ ,  $B = 19.4$ )

Suitable end uses: Blankets, winter coats

#### EXAMPLE 4

Fibrous web of viscose staple an cotton waste  
Specific weight:  $\gamma = 1.53$ , weight  $G = 400$  g/sq.m  
Binding thread: cotton ply yarn Nm 85/2 (T = 211.76  
den.)  
One-bar stitch construction chain stitch  
Wale set: 40 per 10 cm  
Course set:  $N \geq 91.7$  per 10 cm  
( $m = 0.4$ ,  $\alpha = 0.4$ ,  $B = 10.07$ )

Suitable end uses: Packaging materials, industrial fabrics

#### EXAMPLE 5

35 Fibrous web of viscose/polypropylene staple blend,  
two colors (the upper face layer in one color, the lower  
back layer in the other color) weight  $G = 300$  g/sq.m  
Specific weight  $\gamma = 1.52 + 0.95/2 = 1.235$   
Two-bar stitch construction sateen + sateen, oppo-  
site  
Binding thread: Polyamide filament yarn  $T = 90$  den.  
on both bars  
Wale set: 60 per 10 cm  
Course set:  $N \geq 88.9$  per 10 cm  
( $m = 0.4$ ,  $\alpha = 0.2$ ,  $B = 28.45$ )

Suitable end uses: bedspreads, blankets

#### EXAMPLE 6

50 Two component fibrous web: non-shrink material  
(wool) in the upper layer, shrink material (Rhoval) in  
the lower layer total weight  $G = 240$  g/sq.m  
Specific weight:  $\gamma = 1.36 + 1.40/2 = 1.38$   
One-bar stitch construction, chain stitch  
Binding thread: polyamide filament yarn  $T = 90$  den.  
Wale set: 30 per 10 cm  
Course set:  $N \geq 99.3$  per 10 cm  
( $m = 0.4$ ,  $\alpha = 0.08$ ,  $B = 24.7$ )

Suitable end uses: Corduroy or twill backed cloth  
simulation

#### EXAMPLE 7

65 Fibrous web cotton fibers  
Specific weight:  $\gamma = 1.55$ , weight  $G = 350$  g/sq.m  
Binding thread: texturized polyester filament yarn

$T = 250$  den. for the plain stitch construction; polyamide yarn  $T = 90$  den. for the chain stitch construction  
 Resultant denier  $T = (\sqrt{250} + \sqrt{90})^2/2 = 160$  den.  
 Wale set: 50 per 10 cm  
 Course set:  $N \geq 97.3$  per 10 cm  
 $(m = 0.4, \alpha = 0.3, B = 12.98)$

What is claimed is:

1. A quilted fabric comprising a fibrous web fill and a reinforcing thread network applied in a warp knit system having a plurality of wales and courses, wherein the number of courses per 10 cm being at least equal  $N$ ,  $N$  being determined by the equation

$$N = \frac{7589.46}{\sqrt{T}} + 100B \left(1 - \sqrt{1 + \frac{151.79}{B \cdot \sqrt{T}}}\right)$$

where  $B$  is determined by the equation

$$B = \frac{2.88 \cdot G}{T \cdot m \cdot \gamma (0.483 + \alpha)}$$

wherein

$G$  = specific weight in g/sq.m of the fibrous web to be processed

$T$  = binding thread titre in denier

$\gamma$  = specific gravity in g/cu.cm of the fibers in the web

$m$  = the filling coefficient constant defined as the ratio between the sum of fiber cross section areas in a stitch loop and the total area confined by the stitch loop equalling 0.40

$\alpha$  = the constant relating to machine operation a fibrous web weight of up to 200 g/sq.m  $\alpha$  equals zero while with a fibrous web of weight in the range of 200 to 600 g/sq.m,  $\alpha$  is determined by the equation  $\alpha = 0.002 \cdot G - 0.400$ .

2. The fabric according to claim 1 wherein said courses are not less than 80 per 10 cm.

3. The fabric according to claim 1 wherein said knit system comprises a chain stitch having a front loop formed of a double thread and a back loop formed of a single thread.

4. The fabric according to claim 3 wherein said wales are arranged in parallel with each other and binding points form each course and are arranged in parallel rows transversely to said wales.

5. The fabric according to claim 3 wherein said knit system is a combination of chain and tricot stitch, having said front loop formed with two threads, and said back loop formed with one thread, the interconnecting thread between tricot stitches being formed with the

20

$$N = \frac{7589.46}{\sqrt{T}} + 100B \left(1 - \sqrt{1 + \frac{151.79}{B \cdot \sqrt{T}}}\right)$$

25 where  $B$  is determined by the equation

$$B = \frac{2.88 \cdot G}{T \cdot m \cdot \gamma (0.483 + \alpha)}$$

30 wherein

$G$  = specific weight in g/sq.m of the fibrous web to be processed

$T$  = binding thread titre in denier

$\gamma$  = specific gravity in g/cu.cm of the fibers in the web

$m$  = the filling coefficient constant defined as the ratio between the sum of fiber cross section areas in a stitch loop and the total area confined by the stitch loop equalling 0.40

$\alpha$  = the constant which with the fibrous web weight up to 200 g/sq.m  $\alpha$  equals zero while the fibrous webs of weight range of from 200 to 600 g/sq.m  $\alpha$  is determined by the equation

$$\alpha = 0.002 \cdot G - 0.400$$

45 9. The method according to claim 8 including the step of tensioning the warp threads to a predetermined level whereby the binding points between front and back loops is formed in a plane parallel to and substantially at one face of the fabric.

50 10. The method according to claim 8 wherein the number of courses stitches is not less than 80 per 10 cm.

\* \* \* \* \*

55

60

65

back loops.

6. The fabric according to claim 1 having front and back loops in said warp knit system which are interconnected in a series of binding points, the binding points 5 of said front and back loops being located along a plane substantially parallel to and adjacent to one face of said fabric.

7. The fabric according to claim 6 wherein the cross sectional area of the fabric above said plane is substantially smaller than the cross sectional area below said plane.

10 8. In the method of forming a quilted fabric having a fibrous web fill reinforced with network of warp threads knitted in a plurality of wales and courses having 15 a front and back loops interconnected in a series of binding points, the improvement comprising the step of forming the fabric with the number of courses is at least equal to  $N$ ,  $N$  being defined by the equation

$$N = \frac{7589.46}{\sqrt{T}} + 100B \left(1 - \sqrt{1 + \frac{151.79}{B \cdot \sqrt{T}}}\right)$$